

## UNITED STATES PATENT OFFICE

1,937,103

## PENCIL SHEATH COMPOSITION

Jorgen E. Thomsen, Jersey City, N. J., assignor  
to Joseph Dixon Crucible Company, Jersey  
City, N. J., a corporation of New Jersey

No Drawing. Application December 12, 1931  
Serial No. 580,739

7 Claims. (Cl. 106—40)

The invention relates to an improvement in plastic compositions for pencil sheaths and similar articles. This application is a continuation in part of my copending application, Serial No. 5 492,370 filed October 30, 1930.

It has been proposed heretofore to substitute for the usual wood sheath for "lead" and other pencils a sheath composed of a self-hardening plastic compound. Up to the present time, however, so far as I am aware, no practical compound has been disclosed, because the requirements of the art are so varied and conflicting. For example, the sheath produced must be initially so constituted that it can be extruded from a suitable machine while it is in a plastic condition; it must be capable of surrounding, and upon drying, of contracting and firmly gripping the "lead" or other marking material; it must be capable of being easily and smoothly cut by a knife or pencil sharpener; it should have a substantially smooth exterior for the application of a coating or finishing material such as japan or varnish, should one be required; and in general, the pencil sheath composed of the plastic compound must resemble the natural wood sheath in all its qualities as nearly as possible. Not only must the composition sheath meet these practical requirements, it must also meet the commercial requirement of being manufactured at a 10 price permitting it to compete with wood sheaths.

One reason why the plastic compositions heretofore proposed for pencil sheaths have not met all the requirements is that they have shrunk or contracted too much on drying and the pencil sheaths composed of them have warped and twisted. The principal object of the present invention is to produce a composition pencil sheath which will not only meet the practical requirements set forth above but will also have the additional advantage that the pencil composed of the new compound will remain straight and not warp or twist.

The improved composition for pencil sheaths contains several ingredients which have not heretofore been proposed for this purpose and which, combined with the usual pencil sheath composition ingredients, produce the improved pencil sheath. Pencil sheath compositions in general contain a fiber or fibrous material, such as asbestos, a fine cellulose material such as wood

flour, a bonding agent such as casein or viscose, a solvent and plasticizing agent for the casein, if the latter is used, and usually a coloring matter.

I have discovered that one of the reasons why composition pencil sheaths as heretofore compounded become warped or twisted is the fact that some of the ingredients used have required too much water to make the composition extrusible. This fact led me to search for equivalent ingredients which are non-absorbent, or substantially so, and which can be either used with or substituted for the former water-absorbing ingredients. For example, a pencil sheath composition composed largely of finely powdered cellulose, such as wood flour, is highly water absorptive, whereas the fibrous coating of certain cereals, such as rice and maize products, and fibers, such as those obtained from cocoanut hulls, cornstalks, sugarcane stalks and the like, are substantially non-absorbent. By suitably 10 comminuting the rice hulls and/or the other substantially non-absorbent fibers and mixing them in various proportions with the cellulose flour, there can be produced a non-warping and non-twisting pencil sheath. I have also discovered that this new mixture of powdered cellulose and finely comminuted non-absorbent fibrous material can be bonded in an improved manner by the use of a stable water-soluble compound, such as casein, or preferably, a mixture of casein 15 and a stable water-soluble cellulose compound, such as an alkyl derivative of cellulose. These alkyl cellulose compounds are at the present time, available in the open market and are water-soluble binding agents advantageously used in my 20 composition. They may be prepared, for instance, in the manner described in the patents to Lilienfeld Nos. 1,188,376 and 1,505,043 and numerous others. However, it is more convenient to purchase the alkyl cellulose binding agent 25 from a manufacturer thereof. Although an alkyl cellulose is the preferred bonding agent, its market price sometimes prevents its use, in which case it may be partly or wholly replaced by casein.

Viscose has been proposed as a bonding agent 30 for pencil sheath compositions, but I prefer not to use viscose because it is not stable. It begins to harden irreversibly at 70° F., and slowly decomposes even at low temperatures, so that unusual precautions must be taken in preparing it 35

as a bonding agent, and it eventually loses its bonding characteristics in the composition.

By way of example of the preferred embodiment of my invention, I give the following specific formula:—

|    | Ingredient                  | Percentage<br>(by weight) |
|----|-----------------------------|---------------------------|
| 10 | Alkyl cellulose binder..... | 2                         |
|    | Casein.....                 | 17                        |
|    | Lime.....                   | 2                         |
|    | Sodium fluoride.....        | 2.5                       |
|    | Turkey red oil.....         | 4                         |
|    | Wood flour.....             | 54                        |
|    | Comminuted rice hulls.....  | 18.3                      |
| 15 | Coloring matter.....        | .2                        |
|    |                             | 100                       |

The preferred composition for pencil sheaths given above may be compounded in the following manner:—The alkyl cellulose is dissolved in four times its weight of boiling water, and the casein is mixed with about 125 parts of cool water. To the mixture of alkyl cellulose and casein is added the lime mixed with about 50 parts of water, and then the sodium fluoride mixed with about 50 parts of water is added. The whole mixture is thoroughly stirred until the mass is in plastic condition. The turkey red oil and the color are next thoroughly stirred into the mass, and then a mixture of the wood flour and the comminuted rice hulls is added and the mass stirred until the composition is homogeneous. In this condition the plastic composition can be extruded from the machines usually employed for the purpose of producing composition sheath pencils.

If the price of alkyl cellulose is too high for use in making the preferred form of pencil sheath, an excellent substitute pencil sheath, very slightly or not at all inferior in practical qualities to the preferred form, can be made from the following ingredients:—

| 45 | Ingredient           | Percentage<br>(by weight) |
|----|----------------------|---------------------------|
|    | Casein.....          | 18                        |
|    | Lime.....            | 2                         |
|    | Sodium fluoride..... | 2.5                       |
|    | Turkey red oil.....  | 5                         |
| 50 | Wood flour.....      | 54                        |
|    | Rice hulls.....      | 18.3                      |
|    | Coloring matter..... | .2                        |

The foregoing composition can be compounded in substantially the same manner described for the preferred composition.

Casein is a granular powder, it is therefore necessary to plasticize it so as to convert it into a bonding material. This can be done by mixing it with a basic hydroxide, such as lime or ammonia, or with a salt, such as sodium fluoride or sodium phosphate. If it is desired to substitute ammonia for the sodium fluoride or sodium phosphate, then it is desirable to add a preservative and strengthening agent, such as hexamethylene-tetramine or phthalic anhydride. From one to two per cent of these preservative and strengthening

agents is sufficient. The turkey red oil acts as a softening agent for the casein. Soap or rubber substitute, that is, sulphonated oil, may advantageously be substituted for the turkey red oil.

The proportions of the wood flour or other powdered cellulose and the comminuted rice hulls or other fibrous material may vary considerably. I have found, however, that a non-warping and non-twisting composition pencil sheath can hardly be produced if a less proportion than ten per cent of rice hulls or equivalent fibrous material is used in the composition. And on the other hand, if too great a proportion of rice hulls or similar fibrous material is used, then the composition pencil sheath loses in appearance and is also likely to be tougher and not so easily cut by the knife or the pencil sharpening machine. Accordingly, I have found that it is not desirable to use more than twenty or twenty-five per cent of rice hulls or equivalent fibrous material.

The addition of the coloring matter to the mixture is optional.

What I claim is:—

1. A pencil sheath composition comprising a 100 major quantity of wood flour, a minor quantity of a substantially non-water absorbent, comminuted cellulosic fibrous material, and a water-soluble binder.

2. A pencil sheath composition comprising a 105 major quantity of a finely comminuted woody material as its chief ingredient, a minor quantity of finely comminuted substantially non-water absorbent cellulosic fibrous material, and a water-soluble cellulose compound as a binder therefor. 110

3. A pencil sheath composition comprising a major quantity of wood flour as its chief ingredient, about 10 to 25% of a substantially non-water absorbent, finely comminuted cellulosic material, and a water-soluble binder. 115

4. A pencil sheath composition comprising a major quantity of wood flour, about 10 to 25 percent of comminuted rice hulls, and a water-soluble cellulose compound as a binder.

5. A pencil sheath composition comprising the 120 following ingredients in substantially the given percentages by weight: alkyl cellulose binding agent 2%, casein 17%, lime 2%, sodium fluoride 2.5%, turkey red oil 4%, wood flour 54%, comminuted rice hulls 18.3% and coloring matter .2%. 125

6. A pencil sheath composition including a major quantity of a finely comminuted cellulosic material having marked water absorbing properties and a minor quantity of a finely comminuted cellulosic material of greatly less water absorbing properties to reduce the tendency of the pencil sheath to warp, twist and shrink. 130

7. A pencil sheath composition including a major quantity of a finely comminuted cellulosic material having marked water absorbing properties and a lesser quantity, amounting to about 10 to 25% of the total solids, of a finely comminuted cellulosic material of greatly less water absorbing properties to reduce the tendency of the pencil sheath to warp, twist and shrink. 135

JORGENSEN THOMSEN. 140